

## UNITED STATES PATENT OFFICE

2,532,437

DYEING ACRYLONITRILE POLYMERS BY  
APPLYING AN INSOLUBLE AZO DYESTUFF  
AND THEN HEATINGRalph B. Baker, Springfield, Pa., assignor to  
American Viscose Corporation, Wilmington,  
Del., a corporation of DelawareNo Drawing. Application March 15, 1949,  
Serial No. 81,635

7 Claims. (Cl. 8—4)

2

This invention relates to an improved method of dyeing acrylonitrile polymers.

Considerable difficulty is encountered in dyeing the acrylonitrile polymers to deep, fast shades by the conventional dyeing processes. For example, when fibers, yarns, fabrics, or other shaped articles comprising the acrylonitrile polymers are treated with an aqueous dyebath containing a cellulose acetate type dyestuff (sometimes referred to as suspension or dispersal dyes, i. e., insoluble anthraquinone and azo dyes which are applied to cellulose acetate from aqueous dispersion), in the conventional manner of dyeing cellulose acetate, the acrylonitrile polymer articles are merely tinted or dyed to extremely light shades. Moreover, the dyeings do not exhibit good fastness.

An object of the present invention is to provide an improved process for dyeing articles comprising an acrylonitrile polymer to deep, fast shades. Another object is to provide a process for dyeing the acrylonitrile polymers with a dyebath comprising aqueous suspensions of certain azo dyestuffs. A further object is to provide a method for dyeing the acrylonitrile polymers, which does not require the use of special dyeing assistants comprising swelling agents or solvents for the polymer. Other objects will appear hereinafter. I have found that the articles comprising acrylonitrile polymers can be colored by the dyestuffs aforementioned and that the depth of shade and fastness of the dyeings obtained can be markedly improved if, subsequent to the dyeing operation and drying of the dyed article, the article is heated at an elevated temperature of from 120 to 125° C., for at least one hour.

The dyestuffs which are useful in dyeing the acrylonitrile polymers comprise azo aniline derivatives as set forth in the example.

The article comprising the acrylonitrile polymer is treated with the dyebath in the usual manner, using various quantities of dyestuff, with different dyebath ratios and temperatures of the bath, depending on the polymer being dyed, and after the dyeing operation, the article is dried and then baked, as previously explained. The baking to which the dyed article is subjected in the after-treating step serves to fix the dyestuff and results in a marked improvement in the extent of penetration of the dye through the article as evidenced by examination of the cross-section, in the intensity of the color, and in the fastness. The articles dyed and after-treated in accordance with this invention are superior to the control, that is, an acrylonitrile polymer article

dyed in a dyebath of the same composition, under the same conditions, but which is not subjected to the baking after-treatment.

The following example is illustrative of the invention:

## Example

Different lots of yarns of a copolymer of acrylonitrile and vinyl chloride containing 44 mol per cent acrylonitrile in the polymer molecule were dyed in different baths having a dyebath ratio of 1:30 and each containing 2% by weight of one of the dyestuffs listed below, each lot of yarn being treated with one of the baths.

|    |                                                                      |
|----|----------------------------------------------------------------------|
| 15 | Benzene azo-m-phenylenediamine                                       |
|    | p-Dimethyl amino azo benzene                                         |
|    | p-Nitro benzene azo- $\beta$ -hydroxyethyl aniline                   |
|    | p-Nitro benzene azo- $\beta$ -hydroxyethyl-ethylaniline              |
|    | p-Nitro benzene azo- $\beta$ -hydroxyethyl-methylaniline             |
| 20 | line                                                                 |
|    | p-Nitro benzene azo- $\beta$ -hydroxyethyl-o-toluidine               |
|    | p-Nitro benzene azo-di( $\beta$ -hydroxyethyl)-aniline               |
|    | p-Nitro benzene azo dimethylaniline                                  |
| 25 | 2-methoxy-4-nitro benzene azo- $\beta$ -hydroxyethyl aniline         |
|    | 2-methoxy-4-nitro benzene azo- $\beta$ -hydroxyethyl methylaniline   |
|    | 2-methoxy-4-nitro benzene azo- $\beta$ -hydroxyethyl o-toluidine     |
| 30 | 2-methoxy-4-nitro benzene azo- $\beta$ -hydroxyethyl m-toluidine     |
|    | 2-methoxy-4-nitro benzene azo dimethylaniline                        |
|    | 2,4-dinitro benzene azo- $\beta$ -hydroxyethyl aniline               |
|    | 2,4-dinitro benzene azo- $\beta$ -hydroxyethyl-ethylaniline          |
| 35 | line                                                                 |
|    | 2,4-dinitro benzene azo- $\beta$ -hydroxyethyl-methylaniline         |
|    | 2,4-dinitro benzene azo- $\beta$ -hydroxyethyl-o-toluidine           |
| 40 | 2,4-dinitro benzene azo- $\beta$ -hydroxyethyl-m-toluidine           |
|    | 2,4-dinitro benzene azo dimethylaniline                              |
|    | m-Nitrobenzene azo- $\beta$ -hydroxyethyl aniline                    |
|    | O-methoxy benzene azo- $\beta$ -hydroxyethyl aniline                 |
| 45 | 2,6-dichlor-4-nitro benzene azo- $\beta$ -hydroxyethyl-methylaniline |

In each instance, the yarn was entered into the bath at 60° C., and the temperature was raised to the boil, dyeing being continued at the elevated temperature for one hour.

After the dyeing, the yarn withdrawn from each bath was rinsed in cold water, scoured in 0.25% soap solution at 60° C., again rinsed and air-dried. The dried yarn was then baked in an

oven at 120-125° C. for at least one hour, and preferably for about four hours. After the baking treatment the yarns had an intense color and fastness to fading greatly superior to the depth of shade and fastness of the dyed air-dried yarns, prior to the baking after-treatment.

The method of improving the depth of shade and fastness of the dyeing by subjecting the dried, dyed article to the baking treatment appears to be specific to articles comprising polymers containing acrylonitrile in the molecule which have been dyed by means of the particular azo derivatives disclosed herein. Baking did not improve either the depth of shade or the fastness in acrylonitrile polymer articles dyed with other dyestuffs of the type commonly applied to cellulose acetate, and the examination of the cross-section of such articles before and after the baking step did not show improved penetration of the dye as a result of the baking.

The article to be dyed may comprise the acrylonitrile polymer in the form of fibers, yarns, fabrics, filaments, foils, rods, tubings and other shaped articles. The dyeing and baking may be performed on a batch or continuous basis. For example, yarns may be passed continuously through the dyeing, rinsing, scouring, drying, and baking stages and treated on the run, or the article in bulk, for example yarns in skein or other packaged condition, may be treated with the dye-bath and then after withdrawal from the dye-bath, subjected to the baking step.

While various embodiments of the invention have been described in detail for the purpose of illustrating the invention, it is to be understood that changes and variations may be made in practicing the invention, for example in the composition of the acrylonitrile polymer, the concentration of the dye in the bath, etc., without departing from the spirit and scope of the invention as defined in the appended claims.

I claim:

1. A method of dyeing shaped articles comprising an acrylonitrile polymer which comprises treating the article with an aqueous dyebath containing a water-insoluble azo dyestuff selected from the group consisting of

Benzene azo-m-phenylenediamine

p-Dimethyl amino azo benzene

p-Nitro benzene azo- $\beta$ -hydroxyethyl aniline

p-Nitro benzene azo- $\beta$ -hydroxyethyl-ethylaniline

p-Nitro benzene azo- $\beta$ -hydroxyethyl-methylaniline

p-Nitro benzene azo- $\beta$ -hydroxyethyl-o-toluidine

p-Nitro benzene azo-di( $\beta$ -hydroxyethyl)-aniline

p-Nitro benzene azo dimethylaniline

2-methoxy-4-nitro benzene azo- $\beta$ -hydroxyethyl aniline

2-methoxy-4-nitro benzene azo- $\beta$ -hydroxyethyl methylaniline

2-methoxy-4-nitro benzene azo- $\beta$ -hydroxyethyl o-toluidine

2-methoxy-4-nitro benzene azo- $\beta$ -hydroxyethyl m-toluidine  
 2-methoxy-4-nitro benzene azo dimethylaniline  
 2,4-dinitro benzene azo- $\beta$ -hydroxyethyl aniline  
 2,4-dinitro benzene azo- $\beta$ -hydroxyethyl-ethylaniline  
 2,4-dinitro benzene azo- $\beta$ -hydroxyethyl-methylaniline  
 2,4-dinitro benzene azo dimethylaniline  
 m-Nitrobenzene azo- $\beta$ -hydroxyethyl aniline  
 O-methoxy benzene azo- $\beta$ -hydroxyethyl aniline  
 2,6-dichlor-4-nitro benzene azo- $\beta$ -hydroxyethyl-methylaniline

drying the dyed article, and thereafter heating the article at a temperature of from 120 to 125° C., for at least one hour.

2. A method as in claim 1 in which the article comprises a copolymer of acrylonitrile and vinyl chloride.

3. A method as in claim 1 in which the dyestuff is p-dimethylamino azobenzene.

4. A method as in claim 1 in which the dyestuff is p-nitrobenzene azo- $\beta$ -hydroxyethyl aniline.

5. A method as in claim 1 in which the dyestuff is p-nitrobenzene azo- $\beta$ -hydroxyethyl ethylaniline.

6. A method as in claim 1 in which the dyestuff is 2-methoxy-4-nitrobenzene azo- $\beta$ -hydroxyethyl aniline.

7. A method as in claim 1 in which the dyestuff is 2,4-dinitrobenzene azo- $\beta$ -hydroxyethyl aniline.

RALPH B. BAKER.

#### REFERENCES CITED

The following references are of record in the file of this patent:

#### UNITED STATES PATENTS

| Number    | Name    | Date          |
|-----------|---------|---------------|
| 2,080,254 | Dreyfus | May 1, 1937   |
| 2,359,735 | Kienle  | Oct. 10, 1944 |
| 2,461,612 | Olpin   | Feb. 15, 1949 |

#### FOREIGN PATENTS

| Number  | Country       | Date          |
|---------|---------------|---------------|
| 568,037 | Great Britain | Mar. 15, 1945 |

#### OTHER REFERENCES

Amer. Dye. Reporter for October 27, 1941, pp. 575, 578 (article by Heymann).

Rayon and Synth. Textiles for September 1948, pp. 107, 108 (article by Field).

Amer. Dyes Rep. for April 22, 1946, pp. p194, p195.